

[54] SILVER HALIDE EMULSION CONTAINING  
A STABILIZING COMBINATION OF AN  
AZAIDENE AND A  
N,N-DIALKYL-DITHIOCARBAMIC ACID  
ESTER

[75] Inventors: Wolfgang Himmelmann, Opladen;  
Anita Von Konig; Franz Moll, both  
of Leverkusen; Wilhelm Saleck,  
Schildgen, all of Germany

[73] Assignee: AGFA-Gevaert Aktiengesellschaft,  
Leverkusen, Germany

[22] Filed: Aug. 27, 1973

[21] Appl. No.: 392,024

**Related U.S. Application Data**

[63] Continuation-in-part of Ser. No. 176,326, Aug. 30,  
1971, abandoned.

[30] **Foreign Application Priority Data**

Sept. 1, 1970 Germany..... 2043205

[52] U.S. Cl. .... 96/109  
[51] Int. Cl. .... G03c 1/34  
[58] Field of Search ..... 96/109

[56] **References Cited**

UNITED STATES PATENTS

2,716,062 8/1955 Carroll et al..... 96/109  
3,598,598 8/1971 Herz ..... 96/109

*Primary Examiner*—David Klein  
*Assistant Examiner*—Won H. Louie, Jr.  
*Attorney, Agent, or Firm*—Connolly and Hutz

[57] **ABSTRACT**

The stability of photographic silver halide emulsions  
against the formation of fog is improved by addition of  
substituted tetra-azaindene or pentaazaindene and  
N,N-dialkyl-dithiocarbamic acid esters defined herein  
below.

**3 Claims, No Drawings**

SILVER HALIDE EMULSION CONTAINING A  
STABILIZING COMBINATION OF AN AZAIDENE  
AND A N,N-DIALKYL-DITHIOCARBAMIC ACID  
ESTER

This application is a continuation-in-part of our pending U.S. application Ser. No. 176,326 filed Aug. 30, 1971, entitled "A Stabilized Photographic Material," now abandoned.

The invention relates to photographic material comprising at least one silver halide emulsion layer, the stability of which is improved by the addition of N,N-dialkyl-dithiocarbamic acid esters and tetra- or penta-azaindene.

It is well known that photographic emulsions on storage become spontaneously developable without exposure to light. There is normally a detectable amount of the silver salt reduced during development at unexposed areas. This phenomenon is commonly called fog or chemical fog. Fog depends both upon the nature of the emulsion and the conditions of development. For a given emulsion it increases with the degree of development. It is common practice to make accelerated tests of the stability of photographic emulsions by storage at increased temperature or humidity, or both. It is desirable to have emulsions as stable as possible under the condition of high temperature, which may occur in tropical climates. Fog usually appears over the whole area of the light-sensitive layer, but when severe is quite frequently non-uniform.

It is known that certain compounds particularly heterocyclic mercapto or imino compounds have an anti-fogging and stabilizing effect when incorporated into photographic silver halide emulsions and so improve greatly the keeping qualities of the emulsions. Mostly the so-called fog-inhibitors or stabilizers form difficultly soluble or insoluble silver compounds with the silver ions of the photographic emulsion. It is also known that inorganic or organic mercury compounds can be used. Many of these stabilizers however, are of limited utility since they have a desensitizing effect or alter the gradation.

It is among the objects of the invention to provide stabilizers which cause no reduction in the sensitivity at concentrations at which they achieve sufficient stabilization. Another object is to provide a photographic silver halide emulsion that is stable against the production of fog upon storage and stable with respect to the speed and contrast of the emulsion. Other objects and advantages will become apparent from a consideration of the following description and examples.

A photographic material having at least one silver halide emulsion layer has now been found which contains either tetra-azaindene or penta-azaindene and N,N-dialkyl-dithiocarbamic acid esters of the following formula:



wherein

R<sub>1</sub> =

1. aryl, especially a group of the phenyl or naphthyl series, which may be substituted, e.g. with alkyl, alkoxy, alkylthio, nitro, halogen such as fluorine or chlorine, or cyano,
2. alkyl with up to 18, and preferably up to 6, carbon atoms, the alkyl radical may be substituted with cyano, alkylthio, arylthio in particular phenylthio or phenyl such as benzyl or phenylethyl, in which case again the phenyl radical may be substituted as under (1),
3. a heterocyclic group, in particular a ring of the pyrimidine or triazine series, the heterocyclic ring being optionally substituted with halogen such as fluorine or chlorine or aryl, in particular phenyl or naphthyl, which may be substituted as indicated under (1), alkylamino and arylamino, e.g. phenylamino, alkoxy, aroxy, e.g. phenoxy, and the dialkylamino-dithiocarbamic acid group of the above formula;

R<sub>2</sub> = straight chained or branched alkyl with preferably up to 3 carbon atoms which may be substituted, e.g. with cyano.

The compounds listed in the following tables have been found to be especially suitable.

TABLE 1

R<sub>1</sub>—S—CS—N(R<sub>2</sub>)<sub>2</sub>

| Compound number | R <sub>1</sub>                                                                                               | R <sub>2</sub>                   | Melting point           |
|-----------------|--------------------------------------------------------------------------------------------------------------|----------------------------------|-------------------------|
| 1               | 2-nitro-4-chloro-6-hydroxy-phenyl.                                                                           | Methyl                           | 242° C.                 |
| 2               | 2-nitrophenyl                                                                                                | Ethyl                            | 52° C.                  |
| 3               | 2-nitro-6-chlorophenyl                                                                                       | do                               | 78° C.                  |
| 4               | 4-methylthiophenyl                                                                                           | Methyl                           | 114° C.                 |
| 5               | 2,4-dinitrophenyl                                                                                            | do                               | 150° C.                 |
| 6               | 2-chlorophenyl                                                                                               | do                               | 106° C.                 |
| 7               | p-Tolyl                                                                                                      | do                               | 116° C.                 |
| 8               | 2-chloro-6-nitrophenyl                                                                                       | do                               | 152° C.                 |
| 9               | Phenyl                                                                                                       | do                               | 127° C.                 |
| 10              | 3-chlorophenyl                                                                                               | do                               | 76° C.                  |
| 11              | 4-chlorophenyl                                                                                               | do                               | 115° C.                 |
| 12              | 2-nitrophenyl                                                                                                | do                               | 114° C.                 |
| 13              | -CH <sub>2</sub> -CH(CH <sub>3</sub> )-S-C <sub>6</sub> H <sub>5</sub>                                       | Ethyl                            | Oil.                    |
| 14              | 2-methoxybenzyl                                                                                              | Methyl                           | 116° C.                 |
| 15              | -CH <sub>2</sub> -CH-S-C <sub>6</sub> H <sub>5</sub>                                                         | Ethyl                            | Oil.                    |
|                 |                                                                                                              | COOC <sub>2</sub> H <sub>5</sub> |                         |
| 16              | 3-cyano benzyl                                                                                               | Methyl                           | 71° C.                  |
| 17              | 2-cyano benzyl                                                                                               | do                               | 114° C.                 |
| 18              | -CH <sub>2</sub> -S-     | do                               | 48° C.                  |
| 19              | 2,5-dimethylbenzyl                                                                                           | do                               | 60° C.                  |
| 20              | Methyl                                                                                                       | 2-cyanoethyl                     | 89° C.                  |
| 21              | Isobutyl                                                                                                     | Methyl                           | B.P. 64° C. at 0.01 mm. |
| 22              | -CH(CH <sub>3</sub> )-S-CH <sub>2</sub> -C <sub>6</sub> H <sub>5</sub>                                       | do                               | 98° C. decomp.          |
| 23              | -CH(CH <sub>3</sub> )-CH <sub>2</sub> -C <sub>6</sub> H <sub>5</sub>                                         | do                               |                         |
| 24              | -CH <sub>2</sub> -CO-O  | do                               | 220° C. decomp.         |

TABLE 2



| Compound number | R <sub>3</sub> | R <sub>4</sub> | R <sub>5</sub>                                                                                         | Melting point (° C.) |
|-----------------|----------------|----------------|--------------------------------------------------------------------------------------------------------|----------------------|
| 25              | Ethyl          |                | C <sub>1</sub><br> |                      |

TABLE 2—Continued



| Compound number | R <sub>3</sub> | R <sub>4</sub>                                      | R <sub>5</sub>                                                                          | Melting point (°C.) |
|-----------------|----------------|-----------------------------------------------------|-----------------------------------------------------------------------------------------|---------------------|
| 26.             | do             | C <sub>6</sub> H <sub>5</sub>                       | C1                                                                                      | 67-68               |
| 27.             | do             | Cl                                                  | C1                                                                                      | 71                  |
| 28.             | do             | O—CH(CH <sub>3</sub> ) <sub>2</sub>                 | C1                                                                                      | Oil                 |
| 29.             | Methyl         | O—(CH <sub>2</sub> ) <sub>2</sub> —OCH <sub>3</sub> | —S—CS—N(CH <sub>3</sub> ) <sub>2</sub>                                                  | 137                 |
| 30.             | do             | O—CH <sub>2</sub> —CH=CH <sub>2</sub>               | —S—CS—N(CH <sub>3</sub> ) <sub>2</sub>                                                  | 95                  |
| 31.             | do             | O—CH(CH <sub>3</sub> ) <sub>2</sub>                 | —NII—  | 137                 |
| 32.             | Ethyl          | O—C <sub>12</sub> H <sub>25</sub>                   | —S—CS—N(C <sub>2</sub> H <sub>5</sub> ) <sub>2</sub>                                    | 48                  |
| 33.             | Methyl         | O—C <sub>6</sub> H <sub>5</sub>                     | —S—CS—N(CH <sub>3</sub> ) <sub>2</sub>                                                  | 117-118             |
| 34.             | do             | O—CH(CH <sub>3</sub> ) <sub>2</sub>                 | —S—CS—N(CH <sub>3</sub> ) <sub>2</sub>                                                  | 140                 |
| 35.             | do             | O—C <sub>4</sub> H <sub>9</sub>                     | —S—CS—N(CH <sub>3</sub> ) <sub>2</sub>                                                  | 95                  |
| 36.             | do             | O—C <sub>12</sub> H <sub>25</sub>                   | —S—CS—N(CH <sub>3</sub> ) <sub>2</sub>                                                  | 73-74               |

N,N-Dialkyl-dithiocarbamic acid esters are prepared by method known in the literature. Reference may be made to the methods described in Houben-Weyl: "Methoden der organischen Chemie," 4th edition, Volume 9, pages 837-845 and J.Chem.Soc.C., page 466 (1967).

N,N-Dialkyl-dithiocarbamic acid esters together with tetra-, or penta-azaindenes used according to the invention have the advantage over many of the known stabilizers that they do not contain any mercapto groups. The photographic properties such as sensitivity, gradation and clarity are efficiently stabilized by the compounds according to the invention without the graininess or fog being adversely affected.

Many stabilizers which are particularly effective in preventing fogging cause a reduction in the sensitivity of the fresh material, which is often disadvantageous. Other stabilizers which are just sufficiently effective in preventing an increase in fogging cause a substantial and always disadvantageous change in the sensitivity during storage, and this change is in most cases accompanied by a flattening of the gradation. The N,N-dialkyl-dithiocarbamic acid esters and azaindene combination mentioned here have an excellent stabilizing effect both on the gradation and sensitivity so that these properties remain unchanged over long periods of time. The combination of N,N-dialkyl-dithiocarbamic acid esters and azaindenes in the emulsion prevents fog after storage of the unprocessed material in a warm moist atmosphere.

The azaindenes and N,N-dialkyl-dithiocarbamic acid esters to be used according to the invention may be added both to the silver halide layers and to other water-permeable layers, e.g., intermediate layers, protective layers or the baryta layer. These compounds may be added to light-sensitive silver halide emulsions out at any stage of preparation of the emulsion preferably before the after-ripening. The N,N-dialkyl-dithiocarbamic acid esters added may vary within wide limits and quantities of between 0.001 g and 5 g have generally been found sufficient. Particularly advantageous results are obtained when the emulsions contain 1 to 50 mg of the compounds according to the invention per kg of the silver halide emulsion. The tetra-azaindenes and penta-azaindenes, which are stabilizers according to this invention, are described in the article by Birr, Z.Wiss. Phot. 47, 2-58 (1952). It has been

found that the combination of these azaindenes with N,N-dialkyl-dithiocarbamic acid esters of the present invention provides a superior stabilizing effect against moist warm conditions, including after a period of storage. Of particular effectiveness is combination with those tetra-, and penta-azaindenes which are substituted with hydroxyl and amino-groups. Tetra-, or penta-azaindenes used according to this invention may be added in an amount sufficient to provide the advantageous results. An amount of 200 mg of azaindene per kg. of emulsion has been found effective.

The compounds according to the invention are advantageously added in the form of solutions. Suitable solvents are e.g. lower alcohols, tetrahydrofuran, acetone or dimethyl formamide.

The usual silver halide emulsions are suitable for the present invention. These may contain silver chloride, silver bromide or mixtures thereof, optionally with a small silver iodide content of up to 10 mols per cent.

The binder used for the photographic layers is preferably gelatine, although this may be partly or completely replaced by other natural or synthetic binders. Suitable natural binders are e.g. alginic acid and its derivatives such as salts, esters or amides, cellulose derivatives such as carboxymethyl cellulose, alkyl celluloses such as hydroxyethyl cellulose, starch or its derivatives such as ethers or esters or carrageenates. Suitable synthetic binders are e.g. polyvinyl alcohol, partly saponified polyvinyl acetate or polyvinyl pyrrolidone.

The emulsions may also be chemically sensitized, e.g. by adding compounds which contain sulfur at the stage of chemical ripening, for example allyl isothiocyanate, allyl thiourea or sodium thiosulfate. The chemical sensitizers used may also be reducing agents, e.g. the tin compounds described in Belgian Patent Specifications No. 493,464 and 568,687 or polyamine such as diethylene triamine or aminomethyl sulfonic acid derivatives, e.g. according to Belgian Patent Specification No. 547,323.

Noble metals and noble metal compounds, e.g. gold, platinum, palladium, iridium, ruthenium or rhodium, are also suitable chemical sensitizers. This method of chemical sensitization has been described in the article by R. Koslowsky, Z. Wiss. Phot. 46, 65-72 (1951).

The emulsions may also be sensitized with polyalkylene oxide derivatives, e.g. with polyethylene oxide

which has a molecular weight of between 1000 and 20,000 or with condensation products of alkylene oxides and aliphatic alcohols, glycols, cyclic dehydration products of hexitols, alkyl substituted phenols, aliphatic carboxylic acids, aliphatic amines, aliphatic diamines and amides. The condensation products have a molecular weight of at least 700, preferably more than 1000. These sensitizers may, of course, be combined for the purpose of achieving special effects, as described in Belgian Patent Specification No. 537,278 and in British Patent Specification No. 727,982.

The emulsions may also be optically sensitized, e.g. with the usual polymethine dyes such as neutrocyanines, basic or acid carbocyanines, rhodacyanines, hemicyanines, styryl dyes or oxonoles. Sensitizers of this type are described in the work by F. M. Hamer "The Cyanine Dyes and Related Compounds" (1964).

In addition to N,N-dialkyl-dithiocarbamic acid esters and tetra- or penta-azaindenes, the emulsions may contain other known stabilizers.

The emulsions may be hardened in the usual manner, for example with formaldehyde or halo-substituted aldehydes which contain a carboxyl group, such as mucobromic acid, diketones, methane sulfonic acid esters, dialdehydes.

The emulsions may also contain color couplers in dissolved or dispersed form.

The stabilizers which we have described may be used in various kinds of photographic emulsions. In addition to being useful in X-ray and other non-optically sensi-

5 the usual salts. The flocculate is redispersed in warm water, the required quantity of ripe gelatine containing sulfur is added and the emulsion is ripened to optimum sensitivity in the presence of gold(I)-thiocyanate complexes and sodium thiosulfate.

6 Before the emulsion is heated to the ripening temperature, it is divided into 17 portions. The first portion is ripened without additive, whilst the other portions are treated with one of the compounds shown in the table below.

10 After chemical ripening, 200 mg of 4-hydroxy-6-methyl-1,3,3A,7-tetraazaindene as stabilizer, 600 mg of saponin as wetting agent and 10 ml of 10 % aqueous solution of formaldehyde are added, the amounts being in each case based on 1 kg of emulsion.

15 The samples are then cast on a cellulose acetate support and dried, exposed in a sensitometer behind a grey step wedge and developed in a developer of the following composition at 20°C for 7 minutes and 16 minutes:

20

|  |                                 |        |
|--|---------------------------------|--------|
|  | Sodium sulfite sicc.            | 70,0 g |
|  | borax                           | 7,0 g  |
|  | hydroquinone                    | 3,5 g  |
|  | p-monomethylaminophenol sulfate | 3,5 g  |
|  | sodium citrate                  | 7,0 g  |
|  | potassium bromide               | 0,4 g  |
|  | made up with water to 1 litre   |        |

25

20 The results of the sensitometric tests are shown in the following table.

30

Table 3

| Compound No. | Quantity in mg | 7 min. development |      |      | 16 min. development |      |      |
|--------------|----------------|--------------------|------|------|---------------------|------|------|
|              |                | time S             | γ    | fog  | time S              | γ    | fog  |
| control      | —              | —                  | 0,95 | 0,16 | —                   | 1,35 | 0,22 |
| 1            | 2              | —0,5°              | 1,00 | 0,11 | —0,5°               | 1,35 | 0,14 |
| 2            | 8              | ±0°                | 1,00 | 0,14 | ±0°                 | 1,40 | 0,16 |
| 4            | 6              | ±0,5°              | 0,90 | 0,14 | ±0°                 | 1,30 | 0,18 |
| 5            | 3              | —0,5°              | 0,80 | 0,14 | ±0°                 | 1,40 | 0,18 |
| 13           | 10             | —0,5°              | 0,90 | 0,14 | —0,5°               | 1,20 | 0,18 |
| 15           | 6              | —0,5°              | 1,05 | 0,14 | —0,5°               | 1,40 | 0,18 |
| 20           | 10             | ±0°                | 1,05 | 0,14 | ±0°                 | 1,45 | 0,18 |
| 21           | 3              | ±0°                | 0,95 | 0,14 | ±0°                 | 1,40 | 0,19 |
| 23           | 5              | ±0°                | 1,05 | 0,13 | +0,5°               | 1,40 | 0,18 |
| 24           | 10             | ±0°                | 0,80 | 0,14 | +±0°                | 1,20 | 0,18 |
| 25           | 3              | ±0°                | 0,90 | 0,10 | +0,5°               | 1,40 | 0,14 |
| 26           | 3              | —0,5°              | 0,85 | 0,10 | ±0°                 | 1,20 | 0,13 |
| 27           | 3              | —0,5°              | 0,80 | 0,10 | —0,5°               | 1,25 | 0,12 |
| 28           | 3              | —0,5°              | 0,85 | 0,10 | —0,5°               | 1,35 | 0,14 |
| 31           | 6              | ±0°                | 0,80 | 0,11 | —0,5°               | 1,20 | 0,15 |
| 34           | 3              | +0,5°              | 0,85 | 0,10 | ±0°                 | 1,15 | 0,13 |

3° DIN = 1 shutter step  
S = sensitivity

tized emulsions they may also be used in orthochromatic, panchromatic and infrared-sensitive emulsion. They may also be used for emulsions suitable for use in the silver salt diffusion process for colorphotographic emulsions and for photographic materials for the silver dye bleach process.

The following Examples illustrate the invention:

#### EXAMPLE 1

A very highly sensitive silver iodobromide emulsion containing 6 mols per cent of silver iodide is prepared in the usual manner, the silver nitrate solution being poured into a solution which contains gelatine in addition to KBr and KI. The emulsion is flocculated with ammonium sulfate in a known manner and freed from

55 5 A highly sensitive silver iodobromide emulsion containing 5 % of silver iodide is prepared in the usual manner, the silver nitrate solution being run into a solution which contains gelatine in addition to KI and KBr. The emulsion is flocculated in a known manner with

60 ammonium sulfate and freed from the soluble salts by washing. The flocculate is redispersed in warm water, the required quantity of ripe gelatine containing sulfur is added, and the emulsion is ripened to the optimum sensitivity in the presence of gold(I)-thiocyanate complexes and sodium thiosulfate.

65 200 mg of 4-hydroxy-6-methyl-1,3,3a,7-tetraazaindene as stabilizer, 600 mg of saponin as wetting agent and 10 ml of a 10 % aqueous solution of for-

maldehyde are then added to the emulsion, the amounts being in each case based on 1 kg of emulsion. The emulsion is then divided into 18 portions. No additive is added to the first portion and the other portions contain 5 mg/kg of the compounds shown in the following table.

The emulsions are cast on a layer support of cellulose acetate, dried and exposed and developed as described above. Some of the samples are stored at 60°C for 3 days and developed at 20°C for 16 minutes.

The results of the sensitometric test are shown in the following table. This shows that a definite fog stabilizing effect is observed even in the heating cupboard. The substances may therefore be added both before ripening and after chemical ripening as casting additives to achieve a distinct improvement in the fog of the emulsion.

5



10 and with 20 mg of the ortho-chromatic sensitizer:

15



Table 4

| Compound No.          | Development time<br>7 minutes |      |      | Development time<br>16 minutes |      |      | 3 days' heating<br>16 minutes |      |      |
|-----------------------|-------------------------------|------|------|--------------------------------|------|------|-------------------------------|------|------|
|                       | S                             | γ    | Fog  | S                              | γ    | Fog  | S                             | γ    | Fog  |
| control (no additive) | control                       | 0.91 | 0.22 | control                        | 1.13 | 0.30 | control                       | 1.12 | 0.35 |
| 1                     | +1.0°                         | 1.05 | 0.15 | +0.4°                          | 1.19 | 0.21 | -0.5°                         | 1.18 | 0.25 |
| 2                     | +1.0°                         | 0.92 | 0.11 | ±0°                            | 1.12 | 0.20 | +0°                           | 1.13 | 0.21 |
| 4                     | ±0°                           | 0.96 | 0.20 | -0.5°                          | 1.17 | 0.25 | +1.0°                         | 1.19 | 0.30 |
| 5                     | ±0°                           | 0.80 | 0.18 | ±0°                            | 0.92 | 0.21 | ±0°                           | 0.98 | 0.28 |
| 13                    | ±0°                           | 1.06 | 0.21 | ±0°                            | 1.10 | 0.26 | ±0°                           | 1.10 | 0.31 |
| 14                    | ±0°                           | 1.06 | 0.19 | ±0°                            | 1.18 | 0.26 | +1.0°                         | 1.22 | 0.31 |
| 15                    | ±0°                           | 1.02 | 0.19 | -0.5°                          | 1.12 | 0.27 | ±0°                           | 1.05 | 0.32 |
| 20                    | ±0°                           | 1.07 | 0.20 | ±0°                            | 1.09 | 0.28 | +0.5°                         | 1.11 | 0.31 |
| 21                    | ±0°                           | 1.03 | 0.20 | ±0°                            | 1.10 | 0.28 | -1.0°                         | 1.18 | 0.30 |
| 23                    | +0.5°                         | 1.20 | 0.14 | ±0°                            | 1.22 | 0.24 | ±0°                           | 1.30 | 0.27 |
| 24                    | +0.5°                         | 1.05 | 0.15 | ±0°                            | 1.13 | 0.25 | ±0°                           | 1.13 | 0.30 |
| 25                    | ±0°                           | 0.87 | 0.14 | ±0°                            | 1.25 | 0.24 | ±0°                           | 1.29 | 0.26 |
| 26                    | +0.5°                         | 0.93 | 0.17 | ±0°                            | 1.18 | 0.26 | ±0°                           | 1.23 | 0.29 |
| 27                    | ±0°                           | 0.86 | 0.18 | ±0°                            | 1.22 | 0.27 | -1.0°                         | 1.31 | 0.31 |
| 28                    | ±0°                           | 0.88 | 0.17 | ±0°                            | 1.19 | 0.25 | ±0°                           | 1.29 | 0.28 |
| 31                    | +0.5°                         | 0.80 | 0.15 | ±0°                            | 1.20 | 0.20 | ±0°                           | 1.10 | 0.25 |
| 34                    | ±0°                           | 0.75 | 0.14 | -0.5°                          | 1.10 | 0.16 | ±0°                           | 1.15 | 0.18 |

3° = 1 shutter stop

### EXAMPLE 3

An emulsion as described in Example 1 is divided up so that 1 part serves as comparison example without

40 The quantity is based on 1 kg of emulsion. The emulsion samples are cast on a layer support of cellulose acetate and treated in the same way as described in Example 2. The results are shown in the following table.

Table 5

| com-<br>ound<br>No. | Quantity    | Development time<br>7 minutes |       |      | Development time<br>16 minutes |       |      | 3 days' heating<br>16 minutes |       |      |
|---------------------|-------------|-------------------------------|-------|------|--------------------------------|-------|------|-------------------------------|-------|------|
|                     |             | S.                            | γ     | Fog  | S.                             | γ     | Fog  | S.                            | γ     | Fog  |
| blank               | no additive |                               |       |      | -                              | 0.75  | 0.14 | -                             | 1.10  | 0.20 |
| 1                   | 5 mg        | before after-<br>ripening     | +1.0° | 0.70 | 0.10                           | +0.5° | 1.00 | 0.13                          | -1.0° | 0.90 |
| 1                   | 5 mg        | as casting                    | +1.0° | 0.80 | 0.11                           | ±0°   | 1.10 | 0.16                          | ±0°   | 1.00 |
| 14                  | 5 mg        | before after-<br>ripening     | ±0°   | 0.75 | 0.12                           | ±0°   | 1.15 | 0.14                          | -0.5° | 1.05 |
| 14                  | 5 mg        | as casting                    | ±0°   | 0.85 | 0.13                           | -0.5° | 1.20 | 0.14                          | ±0°   | 1.10 |
| 23                  | 5 mg        | before after-<br>ripening     | +0.5° | 0.90 | 0.12                           | +0.5° | 1.25 | 0.15                          | ±0°   | 1.15 |
| 23                  | 5 mg        | as casting                    | +0.5° | 0.85 | 0.11                           | ±0°   | 1.10 | 0.13                          | +0.5° | 0.90 |
| 25                  | 5 mg        | before after-<br>ripening     | ±0°   | 0.70 | 0.09                           | ±0°   | 1.00 | 0.11                          | +0.5° | 0.95 |
| 25                  | 5 mg        | as casting                    | +0.5° | 0.95 | 0.12                           | ±0°   | 1.30 | 0.15                          | ±0°   | 1.20 |

additive and the other part of the emulsion is treated with compounds according to the invention either at the stage of after-ripening or when the emulsion is ready for casting. All the emulsion samples are panchromatically sensitized with 40 mg of the panchromatic sensitizer of the formula:

65 Among other advantages provided by the combination of N,N-dialkyl-dithiocarbamic acid esters and the azaindenes is the prevention of fog after storage of the unprocessed material in a warm moist atmosphere. An emulsion, which does not contain the stabilizer combination, after subjection to moist warm treatment in the

unprocessed state and then developed exhibits an extremely high fog value and/or decreased S and gamma values, particularly when compared with a corresponding emulsion containing the combination of azaindene and N,N-dialkyl-dithiocarbamic acid ester.

Accordingly, it is a feature of the present invention that a silver halide emulsion containing the combination of tetra- or penta-azaindene and N,N-dialkyl-dithiocarbamic acid ester is stabilized against moist warm conditions over a period of time, even though unprocessed.

What is claimed is:

1. A photographic element having at least one light-sensitive silver halide emulsion layer which a stabilizing amount of an azaindene selected from the group consisting of tetra or penta azaindene substituted with hydroxyl or amino groups and a N,N-dialkylthiocarbamic acid ester of the following formula:



5

10

15

20

25

30

35

40

45

50

55

60

65

wherein

$R_1$  represents (1) a phenyl ring, which may be substituted with an alkyl, alkoxy, alkylthio, nitro, halogen or cyano group; or (2) a s-triazine ring, which may be substituted with a halogen, aryl, alkylamino, arylamino, alkoxy, aroxy and the dialkylaminodithiocarbamic acid group;

$R_2$  represents a straight chained or branched alkyl wherein the light-sensitive silver halide emulsion layer contains the dialkylthiocarbamic acid ester in quantities of 5 to 10 milligrams per kilogram of emulsion.

2. The light-sensitive photographic material of claim 1 wherein  $R_2$  represents an alkyl radical having 1 to 3 carbon atoms.

3. The photographic element as claimed in claim 1 wherein 4-hydroxy-6-methyl-1,3,3a,7-tetraazaindene is the azaindene.

\* \* \* \* \*

UNITED STATES PATENT OFFICE  
CERTIFICATE OF CORRECTION

Patent No. 3,854,954

Dated December 17, 1974

Inventor(s) Wolfgang Himmelmann et al

It is certified that error appears in the above-identified patent and that said Letters Patent are hereby corrected as shown below:

Column 2, Table 1, the R<sub>1</sub> substituent of compound 13 should read as follows:  $-\text{CH}_2\text{-CH}(\text{CN})\text{-S-C}_6\text{H}_5$

Column 2, Table 1, the R<sub>1</sub> substituent of compound 22 should read as follows:  $-\text{CH}(\text{CN})\text{-S-CH}_2\text{-C}_6\text{H}_5$

In the Title, "Azaidene" should read -- Azaindene -- .

In the "Inventors": should read -- Anita von König -- .

Signed and sealed this 13th day of May 1975.

(SEAL)

Attest:

RUTH C. MASON  
Attesting Officer

C. MARSHALL DANN  
Commissioner of Patents  
and Trademarks